

June 23, 1925.

1,542,863

E. E. F. CREIGHTON

INSULATED ELECTRICAL CONDUCTOR

Filed Jan. 10, 1918

Fig. 1.



Fig. 2.



Inventor:  
Elmer E. F. Creighton  
by *Albert H. Davis*  
His Attorney.

## UNITED STATES PATENT OFFICE.

ELMER E. F. CREIGHTON, OF SCHENECTADY, NEW YORK, ASSIGNOR TO GENERAL ELECTRIC COMPANY, A CORPORATION OF NEW YORK.

## INSULATED ELECTRICAL CONDUCTOR.

Application filed January 10, 1918. Serial No. 211,111.

*To all whom it may concern:*

Be it known that I, ELMER E. F. CREIGHTON, a citizen of the United States, residing at Schenectady, in the county of Schenectady, 5 State of New York, have invented certain new and useful Improvements in Insulated Electrical Conductors, of which the following is a specification.

My present invention relates to insulated 10 electrical conductors and methods of preparing insulating material and applying it to such conductors.

It is common practice in manufacturing 15 conductors with a covering of fibrous insulating material, such as paper, to first wrap the insulating material around the conductor in successive layers until a covering of the desired thickness has been obtained. The conductor thus covered is then 20 wound upon a reel and placed in a tank where it is subjected to heat treatment in a partial vacuum in order to remove moisture from the insulating material. There is, however, a limit to the amount of moisture 25 which can be removed in this way from paper without destroying a large part of its mechanical strength and thus rendering it unfit for the purpose for which it is used. As a result of this treatment, also, the outer 30 layers of paper on the conductor have more of the moisture removed therefrom than the inner layers so unless the treatment is continued for a much longer time than would be commercially practicable, there must necessarily be a moisture gradient from layer 35 to layer. After treatment in this manner there is still sufficient moisture left in the insulation so that it has an easily measurable ohmic resistance and also a negative 40 temperature characteristic. This negative temperature characteristic is manifested in two ways, first by a decrease in resistance with an increase in temperature and second, by a decrease in puncture voltage with an 45 increase in temperature. Furthermore, such insulation has a higher hysteresis loss with high frequency current than is desirable.

The object of my invention is to provide a 50 method of removing more of the moisture from the insulation than has been possible with the methods heretofore employed without appreciably lowering the mechanical strength of the insulation. A further object of my invention is to provide an insulated conductor which has an improved tempera-

ture characteristic in so far as the puncture voltage is concerned and the insulation of which has a higher resistance and lower hysteresis losses than insulation of the same 60 class previously used.

The usual oil impregnated paper has a decided negative characteristic as already mentioned. By special treatment this negative characteristic decreases and in some cases may even become decidedly positive; that is to say, the puncture voltage increases 65 with the temperature within safe limits of temperature for the fibrous material.

In carrying my invention into effect I 70 treat the insulating material in such a way that a portion of its natural moisture or its moisture of constitution is replaced by an insulating fluid such as oil. By the term "moisture of constitution" I refer to that moisture which forms a part of the cell structure and the removal of which under ordinary conditions, will destroy the continuity of the cell structure or the cohesion between cells and thereby decrease the mechanical strength of the material. This object may be accomplished in a variety of 75 ways. The material may first be dried by ordinary heat and vacuum treatment to as high a degree as possible without greatly weakening it, and then impregnated with 80 oil and subjected to further heat and vacuum treatment. The removal of moisture at this stage may be facilitated by causing a blast of well dried warm air at a few centimeters pressure to pass over the material. The material which is being treated should 85 be so arranged that as large a surface as possible will be exposed in order that the moisture will have a minimum distance to travel through the material before being liberated. I have found that by this treatment a much larger amount of moisture may 90 be removed from the material than with the previously used methods before its mechanical strength is greatly reduced.

Similar results may be obtained by boiling the material in oil. I have found that paper eight mils in thickness, which has been treated by the usual methods, if immersed in oil in separate layers at a temperature of 105° to 110° C. for forty-eight hours will have its puncture voltage increased to 16 kilovolts from a value which may vary from 5 kilovolts to 12 kilovolts. 95 Before the treatment in oil the puncture 100 105 110

voltage of the same paper decreased with increase of temperature from 22° C. to 107° C. about 40%, while after treatment the puncture voltage over the same temperature 5 range increased from 12 kilovolts to 16 kilovolts. When this method is employed the paper or other material should be so arranged that every layer will be in direct contact with the oil in order that the moisture will 10 not have to pass through more than one layer before it is liberated. By this same treatment the insulation resistance of the paper may be measurably increased. The hysteresis losses may also be decreased by a 15 large amount and the danger of puncture thereby greatly lessened as the hysteresis loss plays a most important part in causing puncture.

After the moisture has been removed in 20 this way the insulating material should be kept out of contact with the air to prevent it from absorbing more moisture and air. This may be done by winding it on suitable reels under oil and keeping these reels as 25 well, as the conductor immersed in a tank of oil while it is being wound upon the conductor. An additional advantage in making an insulated conductor in this manner lies in the fact that all air may be excluded 30 from the finished product. When the insulating material is heated in single layers all of the air may easily be removed therefrom, by vacuum treatment, if necessary, and all of the pores therein filled with oil. If the 35 winding operation is also carried out under oil no air will be entrapped between the layers of insulating material. As a result the completed cable will be entirely free from air and free from moisture to an extent which it has been impossible to obtain 40 with the previously used methods of manufacture.

In the accompanying drawing Fig. 1 shows an elevation with portions of the 45 sheath and insulation broken away of a cable constructed in accordance with my invention, and Fig. 2 shows a cross-section of the cable. As indicated in the drawing, a conductor 1 is surrounded by a plurality of 50 layers of insulating material 2 from which the moisture has been thoroughly removed by one of the methods which I have described. Each layer is preferably wound with butt joints between the edges of the 55 strips, the joints between successive layers being broken as indicated. The insulation is covered by the usual lead sheath 3 which is drawn over the insulated conductor as it emerges from the oil bath in which the 60 winding operation is carried on in such a way that there is no opportunity for air or moisture to be absorbed by the insulation or to be entrapped between the sheath and the 65 insulation. In passing through the oil bath all interstices 4 between the strands of the

conductor 1 are also filled with oil. The air being thus entirely excluded from the cable there will be no opportunity for the formation of destructive corona discharges from the conductor when it is employed for high 70 voltage transmission.

What I claim as new and desire to secure by Letters Patent of the United States, is:—

1. An electrical conductor covered with an insulating material, the dielectric strength of which increases with increase of temperature over a range of temperature from 20° C. to 100° C. 75

2. Fibrous material for insulating electrical conductors the puncture voltage of which increases with increase in temperature over a range of temperature from 20° C. to 100° C. 80

3. An electrical conductor covered with a plurality of layers of paper from which the moisture has been removed to such an extent that the puncture voltage increases with increase in temperature over a range of temperature between 20° C. and 100° C. 85

4. The process of preparing fibrous insulating material for electrical conductors which consists in treating separate layers of the same in contact with oil at a temperature of at least 100° C. for a long enough period to remove sufficient moisture 90 to give the material a positive temperature coefficient in regard to the voltage at which it will be punctured over a range of temperature from 20° C. and 100° C. 95

5. Insulating material for electrical conductors, the puncture voltage of which increases with increase in temperature over a range of temperature from 20° C. to 100° C. 100

6. An electrical conductor covered with a fibrous insulating material, the dielectric strength of which increases with increase in temperature over a range of temperature from 20° C. to 100° C. 105

7. The process of preparing insulating material for electrical conductors which consists in treating it while in contact with an insulating fluid at a temperature at least as great as the boiling point of water for a long enough period to remove sufficient moisture to give the material a positive temperature coefficient in regard to the voltage at which it will be punctured over a range of temperature from 20° C. to 100° C. 110 115

8. The process of preparing insulating material for electrical conductors which consists in removing the moisture therefrom to such an extent that it has a positive temperature coefficient in regard to the voltage at which it will be punctured over a range of temperature from 20° C. to 100° C. and at the same time preserving its mechanical strength. 120 125

9. A cable for electrical purposes comprising an electrical conductor, a plurality of layers of fibrous insulating material the 120 125

dielectric strength of which increases with increase in temperature over a range of temperature from 20° C. to 100° C. surrounding said conductor and a protective 5 air tight sheath surrounding said insulating material, the space within said sheath being free from air.

10. The process of manufacturing an insulated electrical conductor which consists in removing moisture from fibrous insulating material, winding the insulating material upon a conductor and preventing the insulating material from coming in contact with the air after the moisture has been removed therefrom and while it is being wound upon the conductor.

11. The process of treating fibrous material which consists in replacing a portion of its moisture of constitution by an insulating fluid.

12. Fibrous material for insulating elec-

trical conductors having a portion of its moisture of constitution replaced by an insulating fluid.

13. An electrical conductor covered with 25 an insulating material in which a portion of the moisture of constitution has been replaced by an insulating fluid.

14. An electrical conductor covered with a plurality of layers of paper in which 30 a portion of the moisture of constitution has been replaced by an insulating fluid.

15. The process of removing moisture from insulating material which consists in impregnating it with an insulating fluid 35 heating the material and then causing dry heated air at a pressure lower than atmospheric to pass over the material.

In witness whereof, I have hereunto set my hand this 8th day of January 1918.

ELMER E. F. CREIGHTON.

**Certificate of Correction.**

It is hereby certified that in Letters Patent No. 1,542,863, granted June 23, 1925, upon the application of Elmer E. F. Creighton, of Schenectady, New York, for an improvement in "Insulated Electrical Conductors," errors appear in the printed specification requiring correction as follows: Page 2, line 69, for the misspelled word "destructure" read *destructive*; lines 75 and 105, claims 1 and 6, for the word "dialectric" read *dielectric*, and line 99, claim 4, for the word "and" read *to*; and that the said Letters Patent should be read with these corrections therein that the same may conform to the record of the case in the Patent Office.

Signed and sealed this 28th day of July, A. D. 1925.

[SEAL.]

KARL FENNING,  
Acting Commissioner of Patents.